

Patented May 29, 1923.

1,457,101

# UNITED STATES PATENT OFFICE.

FRANCIS BRADLEY AND HARRY L. FREVERT, OF PHILADELPHIA, PENNSYLVANIA.

ARMOR PLATE AND PROCESS OF MAKING SAME.

No Drawing.

Application filed June 27, 1922. Serial No. 571,301.

To all whom it may concern:

Be it known that we, FRANCIS BRADLEY and HARRY L. FREVERT, citizens of the United States, residing at Philadelphia, county of Philadelphia, and State of Pennsylvania, have invented a new and useful Improvement in Armor Plates and Processes of Making Same, of which the following is a full, clear, and exact description, reference being had to the accompanying drawings, which form a part of this specification.

Since the equipment of war vessels with iron armor plate designed to resist penetration by cast iron shot, a never ceasing contest has been waged between armor plate and projectiles, the manufacturer of each product endeavouring to overcome the successive improvements made by the manufacturer of the other product. At present the highest type of armor generally in use is the cemented, face-hardened, back-toughened, nickel-chrome plate.

With this plate the object is to break the point of the projectile on a face of intense hardness held together and reinforced by a body of extremely tough, softer metal behind it. Recent improvements made in projectiles by the substitution of a hard-pointed cap for a soft steel cap, upon the point, and by improved methods of manufacture, have produced a projectile whose point is not broken upon the face of the plate, and which, by dislodging the exceedingly hard and correspondingly brittle face, exposes the soft back to ready perforation.

In the penetration of a soft, homogeneous steel plate by a projectile, the anterior surface of the plate is not thrown off as with a carburized, hard-faced plate, but is crowded aside and to the rear, while a certain portion, finding less resistance to movement forward, springs up from the face of the plate in a serrated ring, which is the more pronounced the tougher the material.

We have found that with projectiles of the present improved type, a greater resistance to penetration is offered by a plate which is first treated by known methods to produce a plate having a hardened front with a carburized face and a tough back and which is then drawn at a temperature so high as to remove practically all the brittleness and a large portion of its hardness from the front, while the greater stiffness of the high carbon material forming the

face offers extraordinary resistance to flow. A plate of the type to which our invention is applicable may be produced, for example, by the following process, well known to those skilled in the art: An ingot of any suitable composition is cast, and after reheating is forged or rolled into a plate of a thickness about 20% in excess of the thickness desired for the finished plate. The plate, thus formed, may be reheated and annealed, or reheated to below the critical temperature and cooled either quickly or slowly. The side of the plate intended for the face is then cleaned of all scale and a brick container built around its edges. The container is filled with a suitable carburizing compound, and a similar plate is laid face down upon it, the pair of plates being then heated to a temperature and for a time suitable for penetration of carbon into the face of the plate, to the desired depth and extent, or the plate may be carburized by a gas.

After the carburization of the plate, by the absorption thereby of the desired carbon, the plate is carefully cooled, and freed of scale, the face protected by a carbonaceous covering, reheated to a very low forging temperature and forged to final thickness. The plate is then reheated to a temperature considerably above its critical temperature, quenched, again reheated, but to a less degree than before and again quenched; the plate is then again reheated to a point below its critical temperature, bent and cooled slowly; again reheated to a point well below its critical temperature and quenched. The face of the plate is then heated rapidly to well above its critical temperature, while the back is kept below that temperature and the plate quenched throughout. In this heating operation, the temperature of the plate is raised to above the critical temperature to a depth substantially exceeding the relatively thin carburized face zone and it is this part of the plate, which includes the carburized face and a zone to the rear thereof, which we call the "front."

The above described plate having a hardened front whose face is carburized and a tough back, may be produced by known variations from the above described process, and it will be understood that our process is not limited to the specific process described for producing such a plate; and our

2  
invention, in its broader aspect, does not include any process whatever for producing such a plate as a necessary step of the process.

5 The plate produced by the above known method is then drawn at a temperature not below 500° F. or above 1100° F. We prefer, in the drawing operation, to heat the plate to a temperature of about 650 degrees F. 10 This temperature being distinctly below the critical temperature, the cooling may be effected quickly or slowly.

15 The effect of armor plate so treated upon a projectile is that the point penetrates a certain distance, but the arrest of motion is so rapid that the rear of the shell is upset and broken, in contradistinction to the point, which was formerly broken up.

20 We are aware that attempts have been made to reduce the excessive brittleness of carburized, face-hardened armor plates, with sacrifice of but little of the hardness, by drawing at temperatures up to say 300 degrees F. or thereabouts, but our process 25 differs in that a far greater degree of hardness is relinquished for the corresponding gain in toughness.

This application is a continuation in part of our application for patent for improvement in armor plate and process of making same, filed by us October 29th, 1920, Serial 30 No. 420,483.

Having now fully described our invention,

tion, what we claim and desire to protect by Letters Patent is—

1. The process of so treating armor plate as to render it resistant to penetration, which comprises treating the plate to produce a hardened front with a carburized face and a tough back, and then drawing the plate at a temperature not below 500 degrees F. or above 1100 degrees F., thereby removing from the front practically all its brittleness and a large portion of its hardness, while maintaining the stiffness required to offer extraordinary resistance to displacement.

2. The process of making armor plate comprising treating an armor plate having a hardened front with carburized face and a tough back by drawing said plate at a temperature of between 500 degrees F. and 1100 degrees F.

3. As a new article of manufacture, an armor plate provided with a tough back and a stiff hardened front with a carburized face from which front the normal brittleness has been substantially removed and whose normal hardness has been substantially diminished.

In testimony of which invention, we have hereunto set our hands, at Philadelphia, on this 21st day of June, 1922.

FRANCIS BRADLEY.  
HARRY L. FREVERT.